# EUROPEAN PATENT SPECIFICATION

(11) **EP 1 103 853 B1**
(45) Date of publication and mention of the grant of the patent: **30.10.2002**
(21) Application number: 00203480.9
(22) Date of filing: 05.10.2000
(51) Int. Cl.: G03C 7/413, G03C 7/44, G03C 5/26

(54) **Colour photographic developer concentrate**
Photographisches Farbentwicklerkonzentrat
Révélateur pour la photographie en couleur sous forme concentrée

(30) Priority: 25.11.1999 DE 19956629
(43) Date of publication of application: 30.05.2001
(73) Proprietor: AGFA-GEVAERT, 2640 Mortsel (BE)
(72) Inventor: Tappe, Gustav, 51377 Leverkusen (DE); Körner, Wolfgang, 51373 Leverkusen (DE)

(56) References cited:
- EP-A- 0 528 406
- US-A- 5 891 609

## Description

The developer solution for developing colour photographic materials, in particular for developing colour photographic paper, is prepared from or, in the case of continuous operation, replenished with concentrates which contain the necessary constituents.

It is conventional to provide three different concentrates, as certain constituents of the developer bath are not mutually compatible on extended storage. Thus, for example, one concentrate contains the antioxidant, an auxiliary solvent and an optical brightener, a second concentrate contains the colour developer substance, for example 4-(N-ethyl-N-2-methylsulfonylaminoethyl)-2-methylphenylenediamine sesquisulfate (CD-3) and a third concentrate contains the buffer substance, alkali and a water softener.

There has been no lack of attempts to develop stable, one-part colour developer concentrates as handling errors during preparation or replenishing of a developer solution may consequently be avoided.

Two one-part concentrates are currently commercially available, a) Monoline® RA-4 CD-R from Tetenal, a two-phase concentrate with a solid, undissolved phase deposited at the bottom and b) TriPhase® RA-4 CD-R from Trebla, a three-phase concentrate with undissolved constituents in the middle phase (c.f. also US 5 891 609).

In both cases, the presence of undissolved constituents is disadvantageous for the purposes of handling the concentrate. Especially when preparing the regenerating solution, problems may occur because the undissolved constituents dissolve only poorly. It is also disadvantageous to produce one-part concentrates which, while they contain no undissolved constituents, darken on storage.

The object of the invention was to provide a one-part, aqueous concentrate for a colour developer which contains no undissolved constituents and does not darken on storage.

This object is achieved in that the aqueous concentrate contains at least one colour development agent, at least one auxiliary solvent, alkali, a buffer substance and an antioxidant, wherein the antioxidant is a mixture of 0.1 to 100, preferably of 1 to 25 mmol/l of hydroxylamine and 0.01 to 4, preferably 0.1 to 2 mol/l of one or more substituted hydroxylamines.

In a preferred embodiment, the concentrate contains at most 0.1 mol of sulfate ions/L. The colour developer substance is, for example, added to the concentrate not as the sulfate, as is usual with CD-3, but instead as a phosphate, p-toluenesulfonate, chloride or as the free base.

CD-3 (sesquisulfate) may also be used and the sulfate ions removed by precipitation with metal ions and filtration.

A concentrate for the purposes of the invention is an aqueous preparation, 1 part by volume of which is diluted with 1 to 39 parts by volume of water in order to produce a ready-to-use solution; the concentrate contains at least 50 mmol, preferably 70 to 700 mmol of colour developer substance/L.

The present invention accordingly provides a one-part, optionally multi-phase, colour developer concentrate which contains at least one colour developer substance, an auxiliary solvent, a buffer system and alkali, characterised in that the concentrate contains an antioxidant, wherein the antioxidant is a mixture of 0.1 to 100, preferably 1 to 25 mmol/l of hydroxylamine and 0.01 to 4, preferably 0.1 to 2 mol/l of one or more substituted hydroxylamines.

The concentrate furthermore preferably contains at least one water softener.

Water-soluble organic solvents are in particular used as the auxiliary solvent.

Water-soluble organic solvents which may be considered are those from the range of glycols, polyglycols, alkanolamines, aliphatic and heterocyclic carbonamides, aliphatic and cyclic monoalcohols, wherein 50 to 95 wt.%, preferably 60 to 90 wt.% of the total of water and water-soluble solvent is water.

Suitable water-soluble organic solvents are, for example, carboxylic acid amide and urea derivatives such as dimethylformamide, methylacetamide, dimethylacetamide, N,N'-dimethylurea, tetramethylurea, methanesulfonamide, dimethylethyleneurea, N-acetylglycine, N-valeramide, isovaleramide, N-butyramide, N,N-dimethylbutyramide, N-(2-hydroxyphenyl)acetamide, N-(2-methoxyphenyl)acetamide, 2-pyrrolidinone, ε-caprolactam, acetanilide, benzamide, toluenesulfonamide, phthalimide;
aliphatic and cyclic alcohols, for example isopropanol, tert.-butyl alcohol, cyclohexanol, cyclohexanemethanol, 1,4-cyclohexanedimethanol;
aliphatic and cyclic polyalcohols, for example glycols, polyglycols, polywaxes, trimethyl-1,6-hexanediol, glycerol, 1,1,1-trimethylolpropane, pentaerythritol, sorbitol;
aliphatic and cyclic ketones, for example acetone, ethyl methyl ketone, diethyl ketone, tert.-butyl methyl ketone, diisobutyl ketone, acetylacetone, acetonylacetone, cyclopentanone, acetophenol;
aliphatic and cyclic carboxylic acid esters, for example trimethoxymethane, methyl acetate, allyl acetate, ethylene glycol monomethyl ether acetate, ethylene glycol diacetate, glycerol 1-acetate, glycerol diacetate, methylcyclohexyl acetate, methyl salicylate, phenyl salicylate;
aliphatic and cyclic phosphonic acid esters, for example methylphosphonic acid dimethyl ester, allylphosphonic acid diethyl ester,
aliphatic and cyclic oxyalcohols, for example 4-hydroxy-4-methyl-2-pentanone, salicylaldehyde;
aliphatic and cyclic aldehydes, for example acetaldehyde, propanal, trimethylacetaldehyde, crotonaldehyde, glutaraldehyde, 1,2,5,6-tetrahydrobenzaldehyde, benzaldehyde, benzenepropane, terephthalaldehyde;
aliphatic and cyclic oximes, for example butanone oxime, cyclohexanone oxime;
aliphatic and cyclic amines (primary, secondary or tertiary), for example ethylamine, diethylamine, triethylamine, dipropylamine, pyrrolidine, morpholine, 2-aminopyrimidine;
aliphatic and cyclic polyamines (primary, secondary or tertiary), for example ethylenediamine, 1-amino-2-diethylaminoethane, methyl-bis(2-methylaminoethyl)amine, permethyldiethylenetriamine, 1,4-cyclohexanediamine, 1,4-benzenediamine;
aliphatic and cyclic hydroxylamines, for example ethanolamine, 2-methylethylamine, 2-methylaminoethanol, 2-(diethylamino)ethanol, 2-(2-dimethylaminoethoxy)ethanol, diethanolamine, N-methyldiethanolamine, triethanolamine, 2-(2-aminoethylamino)ethanol, triisopropanolamine, 2-amino-2-hydroxymethyl-1,3-propanediol, 1-piperidineethanol, 2-aminophenol, barbituric acid, 2-(4-aminophenoxy)ethanol, 5-amino-1-naphthol.

Processing conditions, suitable colour developer substances, suitable buffer substances, suitable water softeners, suitable optical brighteners, auxiliary developers, wetting agents, development accelerators and antifogging agents are described on pages 102 to 107 of Research Disclosure 37 038 (February 1995).

Multi-phase means that the concentrate contains two or more liquid phases, but no precipitation. The liquid phases are, for example, an aqueous and an organic phase.

Suitable substituted hydroxylamines are of the formulae (I), (II) and (III). in which
- R₁: means optionally substituted alkyl,
- R₂: means optionally substituted alkyl or optionally substituted aryl and
- n: means 0 or 1
preferably those in which at least one of the residues R₁ and R₂ contains at least one -OH, -COOH or -SO₃H group; in which
- R₃: means an optionally substituted alkyl or optionally substituted acyl group;
in which
- R₄: means an alkylene group optionally interrupted by O atoms and
- m: means a number of at least 2,

The alkyl groups R₁, R₂, R₃, the alkylene group R₄ and the aryl group R₂ may bear further substituents in addition to the stated substitution.

Examples of suitable antioxidants are

(0-3) CH₃CH(CH₃)NHOH

Any phase boundaries which are present disappear on dilution of the concentrate with water to produce the ready-to-use colour developer or regenerator; the ready-to-use developer is one-phase.

For the purposes of storage 200 mL of concentrate are placed in a 250 mL beaker (tall form) and the beaker sealed with an air-tight film (for example PARAFILM "M" ® from American National Can, Chicago). The concentrates are stored for two months at room temperature or 4 weeks at 40°C.

### Examples

### Example 1 (Comparison)

The constituents listed below of a colour developer regenerator are combined in a concentrate (the ready-to-use regenerator is produced from the concentrate by dilution with water):

| One-part, one-phase developer concentrate: | |
|---|---|
| Diethylhydroxylamine, 85 wt.% aqueous solution (DEHX soln.) | 35 mL |
| CD 3, base | 31 g |
| Diethylene glycol | 30 mL |
| Optical brightener W1 | 2 g |
| Ethylenediaminetetraacetic acid (EDTA) | 10 g |
| Potassium carbonate | 60 g |

adjust to pH 13.5 with KOH and make up to 1 litre with water.

The concentrate undergoes distinct darkening on storage.

### Example 2 (Comparison)

| One-part, one-phase developer concentrate: | |
|---|---|
| Antioxidant O-2 | 35 g |
| CD 3, base | 31 g |
| Diethylene glycol | 30 mL |
| Optical brightener W1 | 2 g |
| EDTA | 10 g |
| Potassium carbonate | 60 g |

adjust to pH 13.5 with KOH and make up to 1 litre with water.

The concentrate undergoes distinct darkening on storage.

### Example 3 (Comparison)

| One-part, one-phase developer concentrate: | |
|---|---|
| DEHX soln. | 35 mL |
| Sodium sulfite | 0.5 g |
| CD 3, base | 31 g |
| Diethylene glycol | 30 mL |
| Optical brightener | 2 g |
| Polymaleic acid anhydride, 50% by weight aq. solution | 15 mL |
| Potassium carbonate | 60 g |

adjust to pH 13.5 with KOH and make up to 1 litre with water.

The concentrate undergoes distinct darkening on storage.

### Example 4 (Comparison)

| One-part, one-phase developer concentrate: | |
|---|---|
| DEHX soln. | 35 mL |
| Sodium sulfite | 2 g |
| CD 3, base | 31 g |
| Diethylene glycol | 30 mL |
| Optical brightener | 2 g |
| EDTA | 10 g |
| Potassium carbonate | 60 g |

adjust to pH 13.5 with KOH and make up to 1 litre with water.

The concentrate undergoes distinct darkening on storage.

### Example 5 (according to the invention)

| One-part, one-phase developer concentrate: | |
|---|---|
| DEHX soln. | 35 mL |
| CD 3, base | 31 g |
| Hydroxylammonium sulfate | 0.5 g |
| Diethylene glycol | 30 mL |
| Optical brightener | 2 g |
| EDTA | 10 g |
| Potassium carbonate | 60 g |

adjust to pH 13.5 with KOH and make up to 1 litre with water.

The concentrate is light yellow and does not darken on storage.

### Example 6 (according to the invention)

| One-part, one-phase developer concentrate: | |
|---|---|
| Antioxidant O-2 | 35 g |
| Hydroxylammonium sulfate | 0.5 g |
| CD 3, base | 31 g |
| Diethylene glycol | 30 mL |
| Optical brightener | 2 g |
| EDTA | 10 g |
| Potassium carbonate | 60 g |

adjust to pH 13.5 with KOH and make up to 1 litre with water.

The concentrate is light yellow and does not darken on storage.

### Example 7 (Comparison)

| One-part, multi-phase developer concentrate: | |
|---|---|
| DEHX solution | 60 mL |
| CD 3, base | 45 g |
| Caprolactam | 100 g |
| Triethanolamine | 80 mL |
| Optical brightener | 10 g |
| Diethylenetriamine pentaacetic acid | 40 g |
| Potassium carbonate | 165 g |
| KOH | 42 g |

adjust to pH 11.2 with KOH and make up to 1 L with water.

The upper phase of the concentrate undergoes distinct darkening on storage.

### Example 8 (Comparison)

| One-part, multi-phase developer concentrate: | |
|---|---|
| DEHX solution | 60 mL |
| Sodium sulfite | 2 g |
| CD 3, base | 45 g |
| Caprolactam | 100 g |
| Triethanolamine | 80 mL |
| Optical brightener | 10 g |
| EDTA | 30 g |
| Potassium carbonate | 165 g |
| KOH | 42 g |

adjust to pH 11.2 with KOH and make up to 1 L with water.

The upper phase of the concentrate undergoes distinct darkening on storage.

### Example 9 (according to the invention)

| One-part, multi-phase developer concentrate | |
|---|---|
| DEHX solution | 60 mL |
| Hydroxylammonium sulfate | 0.6 g |
| CD 3, base | 45 g |
| Caprolactam | 100 g |
| Triethanolamine | 80 mL |
| Optical brightener | 10 g |
| EDTA | 30 g |
| Potassium carbonate | 165 g |
| KOH | 42 g |

adjust to pH 11.2 with KOH and make up to 1 L with water.

The upper phase of the concentrate is light yellow and does not darken on storage.

### Example 10

A colour photographic recording material was produced by applying the following layers in the stated sequence onto a layer support of paper coated on both sides with polyethylene. Quantities are stated in each case per 1 m². The silver halide application rate is stated as the corresponding quantities of AgNO₃.

### Layer structure 1

1st layer (substrate layer):
   0.1 g of gelatine
2nd layer (blue-sensitive layer):
   Blue-sensitive silver halide emulsion (99.5 mol% AgCI, 0.5 mol% AgBr, average grain diameter 0.9 µm) prepared from
      0.50 g of gelatine
      0.42 g of yellow coupler GB-1
      0.18 g of yellow coupler GB-2
      0.50 g of tricresyl phosphate (TCP)
      0.10 of stabiliser ST-1
3rd layer (interlayer):
   1.1 g of gelatine
   0.06 g of scavenger SC-1
   0.06 g of scavenger SC-2
   0.12 g of TCP
4th layer (green-sensitive layer):
   Green-sensitive silver halide emulsion (99.5 mol% AgCl, 0.5 mol% AgBr, average grain diameter 0.47 µm) prepared from
      0.40 g of AgNO₃
      0.77 g of gelatine
      0.21 g of magenta coupler PP-1
      0.15 g of magenta coupler PP-2
      0.05 g of magenta coupler PP-3
      0.06 g of colour stabiliser ST-2
      0.12 g of scavenger SC2
      0.23 g of dibutyl phthalate
5th layer (UV protective layer):
   1.15 g of gelatine
   0.03 g of scavenger SC-1
   0.03 g of scavenger SC-2
   0.5 g of UV absorber UV-1
   0.10 g of UV absorber UV-2
   0.35 g of TCP
6th layer (red-sensitive layer):
   Red-sensitive silver halide emulsion (99.5 mol% AgCl, 0.5 mol% AgBr, average grain diameter 0.5 µm) prepared from
      0.30 g of AgNO₃ with
      1.0 g of gelatine
      0.40 g of cyan coupler BG-1
      0.05 g of cyan coupler BG-2
      0.46 g of TCP
7th layer (UV protective layer):
   0.35 g of gelatine
   0.15 g UV-1
   0.03 g UV-2
   0.09 g of TCP
8th layer (protective layer):
   0.9 g of gelatine
   0.3 g of hardener HM
   0.05 g of optical brightener W-1
   0.07 g of vinylpyrrolidone
   1.2 mg of silicone oil
   2.5 mg of polymethyl methacrylate microspheres with an average particle diameter of 0.8 µm

The colour photographic recording material is exposed and processed under the following conditions:

| Step | Time | Temperature |
|---|---|---|
| Development | 27 sec | 39°C |
| Bleach/fixing | 27 sec | 35°C |
| Stabilisation | 54 sec | 33°C |

The colour developers used were ready-to-use developers prepared from the concentrates according to Examples 1 to 9.

### Bleach/fixing bath

| | |
|---|---|
| Ammonium thiosulfate solution, 58 wt.% | 100 mL |
| Sodium disulfite | 5 g |
| Ammonium-iron EDTA, 48 wt.% | 100 mL |

make up with water to 1000 mL, adjust pH value to 6.0 with ammonia or acetic acid.

### Stabilising bath

| | |
|---|---|
| Water | 900 mL |
| Sodium sulfite | 2 g |
| Hydroxyethanediphosphonic acid disodium salt | 4 g |
| Sodium benzoate | 0.5 g |

make up with water to 1000 mL, adjust pH value to 5 with acetic acid.

### Drying

The resultant images exhibited no significant differences with regard to their sensitometric properties.

## Claims

1. One-part, optionally multi-phase, colour developer concentrate which contains at least one colour developer substance, at least one auxiliary solvent, an antioxidant, a buffer system and alkali, **characterised in that** the antioxidant is a mixture of 0.1 to 100 mmol/l of hydroxylamine and 0.01 to 4 mol/l of one or more substituted hydroxylamines.

2. Colour developer concentrate according to claim 1, **characterised in that** it contains one or more water-soluble organic solvents as auxiliary solvent, wherein 50 to 95 wt.% of the total of water and solvent is water.

3. Colour developer concentrate according to claim 1, **characterised in that** the colour developer substance is 4-(N-ethyl-N-2-methylsulfonylaminoethyl)-2-methylphenylenediamine.

4. One-part colour developer concentrate according to claim 1, **characterised in that** the substituted hydroxylamine is of one of the formulae (I), (II) or (III): in which
R₁ means optionally substituted alkyl,
R₂ means optionally substituted alkyl or optionally substituted aryl and
n means 0 or 1;
in which
R₃ means an optionally substituted alkyl or optionally substituted acyl group;
in which
R₄ means an alkylene group optionally interrupted by O atoms and
m means a number of at least 2.

5. One-part colour developer concentrate according to claim 1, **characterised in that** it contains at most 0.1 mol of sulfate ions/L.

6. One-part colour developer concentrate according to claim 1, **characterised in that** it contains at most 0.05 mol of sulfate ions/L.

## Patentansprüche

1. Einteiliges, gegebenenfalls mehrphasiges Farbentwicklerkonzentrat, das wenigstens eine Farbentwicklersubstanz, wenigstens ein Hilfslösungsmittel, ein Oxidationsschutzmittel, ein Puffersystem und Alkali enthält, **dadurch gekennzeichnet, dass** das Oxidationsschutzmittel eine Mischung von 0,1 bis 100 mmol/ℓ Hydroxylamin und 0,01 bis 4 mol/ℓ eines oder mehrerer substituierter Hydroxylamine ist.

2. Farbentwicklerkonzentrat nach Anspruch 1, **dadurch gekennzeichnet, dass** es als Hilfslösungsmittel eines oder mehrere wasserlösliche organische Lösungsmittel enthält, wobei 50 bis 95 Gew.-% der Summe aus Wasser und Lösungsmittel Wasser sind.

3. Farbentwicklerkonzentrat nach Anspruch 1, **dadurch gekennzeichnet, dass** die Farbentwicklersubstanz 4-(N-ethyl-N-2-methyl-sulfonylaminoethyl)-2-methylphenylendiamin ist.

4. Einteiliges Farbentwicklerkonzentrat nach Anspruch 1, **dadurch gekennzeichnet, dass** das substituierte Hydroxylamin einer der Formeln (I), (II) oder (III) entspricht: in der
R₁ gegebenenfalls substituiertes Alkyl,
R₂ gegebenenfalls substituiertes Alkyl oder gegebenenfalls substituiertes Aryl und
n 0 oder 1 bedeuten;
in der
R₃ eine gegebenenfalls substituierte Alkyl- oder gegebenenfalls substituierte Acylgruppe bedeutet;
in der
R₄ eine gegebenenfalls durch O-Atome unterbrochene Alkylengruppe und
m eine Zahl von wenigstens 2 bedeutet.

5. Einteiliges Farbentwicklerkonzentrat nach Anspruch 1, **dadurch gekennzeichnet, dass** es höchstens 0,1 mol Sulfationen/ℓ enthält.

6. Einteiliges Farbentwicklerkonzentrat nach Anspruch 1, **dadurch gekennzeichnet, dass** es höchstens 0,05 mol Sulfationen/ℓ enthält.

## Revendications

1. Concentrat de révélateur chromogène en une seule partie, le cas échéant polyphasique, qui contient au moins une substance développatrice chromogène, au moins un solvant auxiliaire, un antioxydant, un système de tampon et des alcalis, **caractérisé en ce que** l'antioxydant est un mélange d'hydroxylamine à raison de 0,1 à 100 mmoles/l et d'une ou de plusieurs hydroxylamines substituées à raison de 0,01 à 4 moles/l.

2. Concentrat de révélateur chromogène selon la revendication 1, **caractérisé en ce qu'**il contient, à titre de solvant auxiliaire, un ou plusieurs solvants organiques hydrosolubles, dans lequel l'eau représente une quantité de 50 à 95 % en poids du total de l'eau et du solvant.

3. Concentrat de révélateur chromogène selon la revendication 1, **caractérisé en ce que** la substance développatrice chromogène est la 4-(N-éthyl-N-2-méthylsulfonylaminométhyl)-2-méthylphénylènediamine.

4. Concentrat de révélateur chromogène en une seule partie selon la revendication 1, **caractérisé en ce que** l'hydroxylamine substituée répond à la formule (I), (II) ou (III) : dans laquelle
R₁ représente un groupe alkyle le cas échéant substitué,
R₂ représente un groupe alkyle le cas échéant substitué ou un groupe aryle le cas échéant substitué, et
n est égal à 0 ou 1 ;
dans laquelle
R₃ représente un groupe alkyle le cas échéant substitué ou un groupe acyle le cas échéant substitué ;
dans laquelle
R₄ représente un groupe alkylène le cas échéant interrompu par des atomes d'oxygène, et
m représente un nombre au moins égal à 2.

5. Concentrat de révélateur chromogène en une seule partie selon la revendication 1, **caractérisé en ce qu'**il contient une quantité maximale de 0,1 mole d'ions sulfate/l.

6. Concentrat de révélateur chromogène en une seule partie selon la revendication 1, **caractérisé en ce qu'**il contient une quantité maximale de 0,05 mole d'ions sulfate/l.
